

## UNITED STATES PATENT OFFICE

2,258,300

## SOLID LUBRICANT

Arnold J. Morway, Roselle, and John C. Zimmer,  
Hillside, N. J., assignors to Standard Oil De-  
velopment Company, a corporation of Delaware

No Drawing. Application May 6, 1938,  
Serial No. 206,412

8 Claims. (Cl. 252—12)

The present invention relates to improved solid lubricants and more specifically to greases of the type known as block greases used in the lubrication of heavy journal bearings. The lubricant and the method of manufacture will be fully understood from the following description:

Block greases have been used for many years in the lubrication of heavy journal bearings such as locomotive journals. These greases are prepared by saponification of fats or fatty acids at high temperatures in the presence of heavy mineral oils such as cylinder oils, so as to produce a fluid mixture which contains from 25 to 50% of soap and the balance of heavy lubricating oils. The material is held at a high temperature until it is substantially anhydrous, that is to say containing only very little water, usually less than 1%, and frequently about one-half of 1% and cools to a greasy solid. The greases are very hard when cold and have extremely high melting points, in the neighborhood of 300° F. to 400° F. or even 450° F., depending on the amount of soap present and the method by which the melting or softening point is determined. The major fault with the present block greases is that they have a rather grainy structure and do not possess as good lubricating qualities as might be desired, these latter being to some extent sacrificed in order to gain hardness and the high melting point required for the service.

It has been found that the above difficulties can be overcome by the use of a particular ingredient in the manufacture of the grease. This material is a byproduct of the low temperature, low pressure air oxidation of paraffin wax with catalysts. It is known that paraffin wax may be oxidized with air in the liquid phase and in the presence of a catalyst such as barium and manganese soaps at temperatures from 100° to 150° C. and at atmospheric or only slightly elevated pressure to yield a large portion of volatile or distillable fatty acids of the molecular weight range used for soap making. Other compounds are produced in addition to the acids, but the material desired for present purposes is a material of unknown constitution, probably polymerized to a considerable degree so that it is substantially undistillable even under vacuum.

This material may be obtained in various ways from the crude wax oxidation product, but it is preferred to saponify the fatty materials under pressure with aqueous caustic soda, so as to make a fluid material. Alcohol may be added to prevent emulsification. This product is then extracted with naphtha, kerosene or other solvent

in order to remove most of the unconverted wax. The soap solution is then preferably distilled to recover the alcohol and reacidified so that the acids and other organic material collects in a layer above the aqueous solution and this organic layer is decanted and distilled under vacuum, so as to take off substantially all of the material that can be reasonably described as distillable.

The products obtained as a distillate are largely acids of the soap making range, that is containing from 12 to 18 carbon atoms, but it is the residue which is desired for the present purposes. The chemical constitution of this material is not fully understood, but it has been analyzed to some extent with the following results:

|                                                                                                                                                                                                                                                                                                                                                                                                          | Per cent |
|----------------------------------------------------------------------------------------------------------------------------------------------------------------------------------------------------------------------------------------------------------------------------------------------------------------------------------------------------------------------------------------------------------|----------|
| Free acids, about                                                                                                                                                                                                                                                                                                                                                                                        | 30       |
| Esters, lactones, etc.                                                                                                                                                                                                                                                                                                                                                                                   | 65       |
| Unsaponifiable, about                                                                                                                                                                                                                                                                                                                                                                                    | 5        |
| 20 The total mixture has a neutralization value of about 46 mg. KOH per gram. The saponification value when the mixture is refluxed with KOH is about 175 mg. KOH per gram, and when carried out under pressure the value is about 230 mg. KOH per gram. It will be seen that this material is very different from an ordinary fat or wax, and it is also free from aldehydes or aldehydelike compounds. |          |
| 30 The free acid content of the material when roughly separated, for example by solution in alcoholic caustic soda, has the following characteristics:                                                                                                                                                                                                                                                   |          |
| 35 Iodine value mg. per gram                                                                                                                                                                                                                                                                                                                                                                             | 99       |
| 35 Neutralization value mg. KOH per gram                                                                                                                                                                                                                                                                                                                                                                 | 85.5     |
| 35 Saponification value (reflux) in KOH mg. per gram                                                                                                                                                                                                                                                                                                                                                     | 186.9    |
| 35 Saponification value (pressure) do mg. per gram                                                                                                                                                                                                                                                                                                                                                       | 220.5    |
| 40 The average molecular weight of this acidic material is about 626.5 which is, of course, much higher than most of the known fatty acids highly unsaturated and free of aldehydes. The material remaining after removal of free acid has the following characteristics:                                                                                                                                |          |
| 45 Iodine value mg. per gram                                                                                                                                                                                                                                                                                                                                                                             | 82       |
| 45 Saponification value (pressure) per gram                                                                                                                                                                                                                                                                                                                                                              | 115.7    |
| 45 Naphtha soluble per cent                                                                                                                                                                                                                                                                                                                                                                              | 97.5     |
| 45 Naphtha insoluble do                                                                                                                                                                                                                                                                                                                                                                                  | 2.5      |
| 50 Saponifiable do                                                                                                                                                                                                                                                                                                                                                                                       | 92.2     |
| 50 Unsaponifiable do                                                                                                                                                                                                                                                                                                                                                                                     | 8.6      |
| 55 From the above analyses it would appear that the vacuum distillation residue consists of very high molecular weight acids, which are highly unsaturated, together with unsaturated esters                                                                                                                                                                                                             |          |

and other saponifiable material. The material is polymerized and is of higher molecular weight than the wax from which it was obtained.

In making the improved block greases, the above mentioned material which will be referred to in this specification and in the claims as a nondistillable byproduct of the air oxidation of wax, may be used as the sole soap yielding organic material or it may be admixed with other fatty materials such as fats and fatty acids. It is preferred to use a major quantity of this material, however, with only minor amounts of fats or fatty acids; for example, while the equal quantities may be used, it is preferred to use 5 to 10 times as much of the wax oxidation product as of the low molecular weight fat or fatty acid. The wax oxidation byproduct or its mixture with fat or fatty oil is then admixed with lubricating oil, such as a cylinder oil or other viscous lubricating stock. If desired, a part of the cylinder oil may be replaced with petrolatum which also improves the characteristics of the grease. This mixture is melted together by heat to about 160° F., at which temperature aqueous caustic soda is added. The amount of the caustic soda added should be sufficient to saponify all of the low molecular weight fat which may be present and at least 75 to 85% of the wax oxidation product. If desired the alkali added may be sufficient to neutralize all of the acid groups of the wax oxidation byproduct and free acid may be added such as naphthenic acid or the volatile acids produced by the wax oxidation or other fatty acid. This should be added in proportions from .10 to say 10% of the final grease. The mixture is then agitated and the temperature is raised to about 400 or 450° F., so as to bring about the reaction, and heating is continued until a substantially anhydrous material is obtained; that is to say, the water content is reduced below 1%. The material is then withdrawn from the kettle and cooled in pans.

As a specific example of the method of manufacturing the grease, the following may be considered:

25 parts of the nondistillable wax oxidation product described hereinabove were mixed with 2.5 parts of kidney rosin oil and 50 parts of cylinder oil. 20 parts of petrolatum, which had a melting point of 150° F., were then added and the mixture was heated to 160° F., at which temperature the ingredients melted into a more or less homogeneous fluid mass. Caustic soda solution, 20% aqueous NaOH, was then added containing 2.4 parts of dry NaOH, and temperature was raised to 420° F. while agitating. The stirring was continued at this temperature for about 1-2 hours, until the product contained less than 1% water and then was withdrawn and cooled in shallow pans.

The grease was hard but with a smooth and unctuous structure, remarkably free from graininess and had the appearance and feel of a water grease, although it was a dehydrated product and extremely hard. It had a melting point of about 350° F. by the drop method and an A. S. T. M. penetration of 50-100 at 77° F.

The present invention is not to be limited by any theory of the use of the various ingredients, nor to any particular ingredients or proportions thereof, but only to the following claims in which it is desired to claim all novelty inherent in the invention.

We claim:

1. An improved block grease comprising min- 75

eral oil, a small amount of kidney rosin oil and as the main soap ingredient an alkali soap obtained by saponification of a byproduct of wax oxidation obtained by neutralization of the crude oxidation product removal of unconverted wax, reacidification, and non-destructive distillation of the volatile acids under conditions to leave undisintegrated said non-distillable acidic residue byproduct free from acid having not more than 18 carbon atoms and the acids present having an average molecular weight of at least about 600.

2. An improved block grease comprising a heavy mineral oil, a small amount of kidney rosin oil and at least 25% of an alkali soap of a non-volatile acidic material obtained by saponifying a crude oxidation product, removing unconverted wax reacidifying with mineral acid and distilling off the volatile organic acids under high vacuum so as to recover a non-distillable acidic residue the acids present in which have an average molecular weight of at least about 600 and are free from acids having not more than 18 carbon atoms which is used in the preparation of the soap.

25. 3. Product according to claim 2 in which the grease contains a small amount of a soap of a fatty acid.

4. Product according to claim 2 in which the grease comprises about 25 parts of the non-volatile oxidation product, 2½ parts of kidney rosin oil, about 70 parts of heavy hydrocarbons, and caustic soda sufficient to saponify the kidney rosin oil and at least 75% of the oxidation product.

5. Product according to claim 2 in which the oil is a cylinder oil and petrolatum is added thereto.

6. A block grease comprising mineral oil, a small amount of kidney rosin oil and, as the main soap ingredient, an alkali soap of a high molecular weight non-distillable unsaturated polymerized acidic residue obtained as a by-product of wax oxidation, which is free from acids having 18 or less carbon atoms and which is substantially free from unconverted wax, and the acid content of said acidic residue having an average molecular weight of at least about 600.

7. A solid lubricating grease having a hard, smooth, unctuous structure substantially free from graininess, having a melting point of about 350° F., an A. S. T. M. penetration of about 50-100 at 77° F., and containing less than about 1% of water, said grease being made from the following materials using approximately the proportions indicated:

High molecular weight non-distillable polymerized wax-oxidation acidic by-product having a saponification value of about 175 mg. KOH per gram and consisting essentially of about 30% of unsaturated free acids having an average molecular weight of about 626.5 and free from acids having 18 or less carbon atoms, the balance of said acidic by-product being an aldehyde-free mixture of about 65% of esters, lactones, etc. and about 5% of unsaponifiable material.

|                                                      |       |      |
|------------------------------------------------------|-------|------|
| Kidney rosin oil                                     | parts | 25   |
| Cylinder oil                                         | parts | 2.5  |
| Petrolatum (melting point about 150° F.)             | parts | 50   |
| Caustic soda solution (20% concentration) containing | parts | 20   |
| parts of dry NaOH                                    | parts | 2.4  |
| Total                                                | parts | 99.9 |

8. The process of preparing a dehydrated block grease which comprises melting and heating to about 160° F. a mixture of a mineral oil, a small amount of kidney rosin oil and a high molecular weight non-distillable acidic residue obtained as a by-product from the oxidation of paraffin wax, said residue being free from acids having 18 or less carbon atoms but said residue having a free-acid content having an average molecular weight of at least about 600 and said residue having a 10 neutralization value of about 46 mg. KOH per gram, a saponification value, refluxed, of about

175 mg. KOH per gram and a pressure saponification value of about 230 mg. KOH per gram, adding to the above-formed mixture a sufficient amount of aqueous caustic soda solution to saponify at least 75% of the free acid content of the wax oxidation product, agitating, and heating the mixture to about 400° F. to complete the reaction and to dehydrate the product to a water content below 1%.

ARNOLD J. MORWAY.  
JOHN C. ZIMMER.